

# United States Patent

[11] 3,545,525

[72] Inventor **Albertus Antonie Aldenkamp**  
**Emmasingel, Eindhoven, Netherlands**  
[21] Appl. No. **676,642**  
[22] Filed **Oct. 19, 1967**  
[45] Patented **Dec. 8, 1970**  
[73] Assignee **U.S. Philips Corporation**  
**New York, N.Y.**  
**a corporation of Delaware, by mesne**  
**assignments**  
[32] Priority **Oct. 20, 1966**  
[33] **Netherlands**  
[31] **No. 6614748**

[54] **METHOD OF MANUFACTURING**  
**MAGNETICALLY ANISOTROPIC PERMANENT**  
**MAGNETS WITH A CRYSTAL ORIENTATION**  
**2 Claims, No Drawings**

[52] U.S. Cl. .... **164/82;**  
..... **148/31.57, 148/101; 164/122**

[51] Int. Cl. .... **H01f 1/04,**  
..... **H01f 7/02**  
[50] Field of Search. .... **164/82,**  
..... **122, 128, 146; 148/101, 31.57**

[56] **References Cited**  
**UNITED STATES PATENTS**

|                  |               |                            |                  |
|------------------|---------------|----------------------------|------------------|
| <b>2,398,018</b> | <b>4/1946</b> | <b>Linley et al.</b> ..... | <b>164/146X</b>  |
| <b>3,189,957</b> | <b>6/1965</b> | <b>Luteijn</b> .....       | <b>164/82</b>    |
| <b>3,314,828</b> | <b>4/1967</b> | <b>Harrison</b> .....      | <b>148/31.57</b> |

*Primary Examiner—J. Spencer Overholser  
Assistant Examiner—John E. Roethel  
Attorney—Fank R. Trifari*

**ABSTRACT:** An Fe-Co-Ni-Al alloy suitable for continuous casting of crystal oriented magnetically anisotropic permanent magnets containing not more than 0.15 percent of silicon which is continuously cast in a tube and cooled at such a rate as to prevent the formation of a  $\gamma$ -phase.

**METHOD OF MANUFACTURING MAGNETICALLY ANISOTROPIC PERMANENT MAGNETS WITH A CRYSTAL ORIENTATION**

The invention relates to a method of manufacturing crystal oriented magnetically anisotropic permanent magnets consisting of a Fe-Co-Ni-Al alloy containing, in addition to Fe and the usual impurities, approximately 15 to 42 percent of Co, approximately 10 to 20 percent of Ni, approximately 6 to 10 percent of Al, up to 8 percent of Cu and any additions such as, for example, Si, up to 4 percent of Nb, up to 8 percent of Ta, while the content of Nb and/or Ta may be replaced entirely or in part by Ti. The invention also relates to an alloy suitable for the manufacture of crystal oriented magnetically anisotropic permanent magnets.

Such methods are known from Dutch Pat. Specification 109,811 and the Dutch application 289,045 laid open for public inspection. These methods have the great advantage that permanent magnets which have satisfactory magnetic properties (for example,  $H_c \sim 750$  Oe;  $B_r \sim 13500$  G;  $(BH)_{max} \sim 8 \times 10^6$  G. Oe) can be manufactured in a comparatively simple manner by a continuous process. This involves great economic advantages. Moreover, the magnets thus manufactured have a constant quality within small tolerances.

It has been found that with the use of the aforesaid casting methods, the continuous casting process was sometimes interrupted because the solidified alloy clogged in the tube. A tube in which the alloy has once clogged must be replaced. This involves large expenditures for material and mounting.

It has been found that pure  $Al_2O_3$  sintered to compactness is a particularly suitable material for the tube, inter alia because it has the following properties: it does not dissolve in the alloy, it has a high melting point, a low porosity and a high resistance to wear.

Investigations have shown that clogging of the rod in the  $Al_2O_3$  tube may be due to reactions of the solidifying alloy with the wall of the tube.

It is common practice in the manufacture of permanent magnets consisting of a Fe-Co-Ni-Al alloy to provide a quantity of Si lying between approximately 0.15 and 5 percent preferably a quantity lying between 0.2 and 0.4 percent in this alloy. Such an addition prevents the formation of a cubic-face-centered  $\gamma$ -phase besides the already available cubic-space-centered  $\alpha$ -phase during cooling of the alloy after solidification. The presence of this  $\gamma$ -phase detrimentally affects the permanent magnetic properties of the material. If no Si were added, the said  $\gamma$ -phase would actually be formed during cooling and the material would have to be subjected to an additional—and hence cost-increasing—thermal treatment in order to eliminate said  $\gamma$ -phase.

Investigations have shown that the aforesaid reactions between the wall of the tube and the alloy are due to the fact that the  $Al_2O_3$  of this tube wall is more readily attacked with higher silicon content of the alloy. During these experiments, it had been ensured that the alloy was poor in oxides, since these oxides also react with the wall of the tube so that clogging of the rod could also be due to these oxides. Therefore, attempts had to be made to prevent contact between the Si in the alloy and the  $Al_2O_3$  of the wall of the tube. However, the combination of favorable properties found in particular in  $Al_2O_3$  had nevertheless to be maintained in the tube. Moreover, the formation of a  $\gamma$ -phase during cooling of the melt in the tube had to be prevented, since otherwise the aforesaid additional thermal treatment for elimination of this

phase is required. So it seemed that the use of an alloy poor in Si was also impossible.

The invention is based on the discovery that, when using the continuous casting process, the alloy can be cooled in the tube at such a high rate that, even without the addition of Si, the formation of a  $\gamma$ -phase during cooling is prevented. It is then required that at least a given temperature gradient occurs in the  $Al_2O_3$  tube. Such a temperature gradient may be achieved by means of the continuous casting process either by choosing the rate of drawing above a given minimum value, or by cooling the tube sufficiently.

According to the invention, the alloy which is supplied in the molten state at the upper end of an  $Al_2O_3$  tube and is withdrawn in the solid state at the lower end of this tube contains at the most 0.15 percent of Si, while the cooling rate is at least  $0.4^\circ C./sec.$

Experiments have shown that with an alloy containing 0.5 percent of Si, the casting process stagnated after 3 hours, with a content of 0.35 percent of Si after 24 hours and with an Si-content of 0.15 percent after one week. It has been found that no further improvement can be obtained by further reducing the Si-content. A further reduction of the Si-content below 0.15 percent no longer has any influence on the reaction between the alloy and the wall of the tube, which is due to the fact that in this case, other effects, which are dominated at a higher Si-content by the Si-effect, start playing a part.

When the temperature gradient in the tube is chosen to be sufficiently large, i.e.,—so that for a given rate of drawing, the corresponding rate of cooling of the solidified alloy is, for example,  $\frac{1}{2}^\circ C./sec.$  or  $1^\circ C./sec.$ , it has been found that the formation of a  $\gamma$ -phase is prevented.

For example, an alloy consisting of 28 percent by weight of Co, 14 percent by weight of nickel, 8 percent by weight of aluminum, 3 percent by weight of copper, 2 percent by weight of titanium, 0.1 percent by weight of silicon and the balance iron was introduced in molten form into an  $Al_2O_3$  tube having an inner diameter of 18.5 mm. under an argon atmosphere. A bar was drawn from the other end of the tube in which the (100) direction of the crystals were oriented axially at the rate of 7 mm./sec. The temperature gradient within the tube was about  $15^\circ C./min.$  and the cooling rate  $2^\circ C./sec.$

While the invention has been described in connection with a particular example, other modifications will be apparent to those skilled in the art without departing from the spirit and scope of the invention which is defined in the appended claims.

I claim:

1. In the method of manufacturing crystal oriented magnetically anisotropic permanent magnets containing approximately 15 to 42 percent of Co, approximately 10 to 20 percent of Ni, approximately 6 to 10 percent of Al, up to 8 percent of Cu, up to 4 percent of Nb and up to 8 percent of Ta, up to 8 percent of Ti and the balance iron and impurities in which the alloy is supplied in the molten state at the upper end of an  $Al_2O_3$  tube and is withdrawn in the solid state at the lower end of the tube, the improvement comprising supplying alloys containing at the most 0.15 percent of Si, and cooling the alloy in the tube at a rate of at least  $0.4^\circ C./sec.$  to prevent the formation of a  $\gamma$ -phase in the alloy.

2. A method of manufacturing crystal oriented magnetically anisotropic permanent magnets as claimed in claim 1 in which the alloy is cooled in said tube at a rate of about  $\frac{1}{2}$  to  $1^\circ C./sec.$  to prevent the formation of a  $\gamma$ -phase.